

# United States Patent

[19]

Miyauchi et al.

[11] 3,719,769

[45] March 6, 1973

[54] **INSULATED ELECTRIC CABLE HAVING AN EXTERNAL SEMICONDUCTIVE LAYER**

[75] Inventors: Hirokazu Miyauchi; Hironaga Matsubara, both of Osaka, Japan

[73] Assignee: Sumitomo Electric Industries, Ltd., Osaka, Japan

[22] Filed: Oct. 5, 1970

[21] Appl. No.: 77,918

[52] U.S. Cl...174/120 SC, 174/105 SC, 174/110 PM

[51] Int. Cl.....H01b 9/02

[58] Field of Search...174/36, 120 R, 120 SC, 102 R, 174/102 SC, 105 SC, 106 SC, 110 PM, 107, 127

[56] **References Cited**

## UNITED STATES PATENTS

- |           |         |                                   |
|-----------|---------|-----------------------------------|
| 3,259,688 | 7/1966  | Towne et al.....174/127 X         |
| 3,441,660 | 4/1969  | Garner.....174/110 PM X           |
| 3,472,692 | 10/1969 | Setsuya Isshiki.....174/106 SC UX |
| 3,433,891 | 3/1969  | Zysk et al.....174/102 SC X       |
| 3,287,489 | 12/1966 | Huijd, Jr. ....174/102 SC         |
| 3,096,210 | 7/1963  | Boonstra.....174/110 PM UX        |

## FOREIGN PATENTS OR APPLICATIONS

1,103,099 2/1968 Great Britain.....174/102 SC

## OTHER PUBLICATIONS

The Condensed Chemical Dictionary 6th Ed., Reinhold 1961, p. 395. (QD 5 C5 1961 c.12)

Primary Examiner—Bernard A. Gilheany

Assistant Examiner—A. T. Grimley

Attorney—Carothers and Carothers

[57] **ABSTRACT**

An insulated electric cable having an external semiconductive layer with easy stripping qualities for termination wherein the cable is insulated primarily with crosslinked polyethylene or a crosslinked polyethylene copolymer and the external semiconductive layer consists of an ethylene vinyl acetate copolymer containing 25-55 wt-percent vinyl acetate and 2,5-dimethyl-2',5'-di(tertiary butyl/peroxy)-hexane-3 and an inclusion of an electric conductive substance such as carbon black to render the layer semiconductive.

7 Claims, 1 Drawing Figure



PATENTED MAR 6 1973

3,719,769



INVENTORS.  
HIROKAZU MIYAUCHI &  
HIRONAGA MATSUBARA  
By  
CAROTHERS & CAROTHERS  
THEIR ATTORNEYS

## INSULATED ELECTRIC CABLE HAVING AN EXTERNAL SEMICONDUCTIVE LAYER

This invention relates to an insulated cable having an external semiconductive layer, and more particularly to the structure of an insulated cable having an insulation primarily consisting of crosslinked polyethylene or a crosslinked polyethylene copolymer, having an external semiconductive layer.

In the conventional art, when covering the insulating layer of a crosslinked polyethylene insulated cable with an extruded semiconductive layer, wherein low density polyethylene, a copolymer of ethylene and vinyl acetate or a polymer consisting mainly of these substances is used as the base of the insulation layer, to which are further added talc, clay, calcium carbonate and like inorganic fillers, various age resistors, processing aids and the like as required, it is a usual practice to use a composition such as a mixture of a copolymer of ethylene and ethyl acrylate, with dicumyl peroxide and the like AD crosslinking agents and electric-conductive carbon black, or a mixture of a copolymer of ethylene and vinyl acetate, with dicumyl peroxide and the like crosslinking agents, and electric-conductive carbon black for the semiconductor outer layer.

When splicing and treating the end of a crosslinked polyethylene insulated cable having the external semiconductive layer, it is necessary to remove the semiconductive layer of the cable for a certain length from the end thereof. The removal of the semiconductive layer should be complete in this case, and in removing it the insulating layer should be left intact. In recent years, through the development of the art, parts and accessories premolded to the shape of cable joints and terminations have come in handily for the splicing and terminating of crosslinked polyethylene insulated cable having an external semiconductive layer. This method gives a more stable quantity and facilitates a more speedy operation as compared with the conventional treatment methods of wrapping with a tape, heat molding and like means, and the above method is now widely used. In this method, however, it is required that the premolded accessories used should be fitted to the contour of the cable without allowing any electrical faults to exist therebetween. Thus demands are growing for a method to easily strip off the semiconductive layer without damaging the insulating layer in a short period of time than heretofore possible.

When the conventional compositions as abovementioned are used to cover the insulated layer, it is hard and takes time to first strip off the semiconductive coating, and the insulation layer easily marred. Thus none of these compositions satisfy the abovementioned requirements.

The present invention, however, is intended to provide a crosslinked polyethylene insulated cable having a semiconductive layer which can be easily stripped off without leaving a fraction of the semiconductive layer on the surface of the insulating layer nor marring the insulating layer.

The present invention pertains to a crosslinked polyethylene insulated cable having a semiconductive layer which is extruded over the insulating layer, and provides the cable with a semiconductive layer which can be easily stripped off. This semiconductive layer is formed by extruding a composition obtained by mixing

a copolymer of ethylene and vinyl acetate, containing 25-55 wt percent vinyl acetate and desirably in a range, in excess of 0.2 but less than 6.0 wt. parts of 2,5-dimethyl-2', 5'-di(tertiary butyl peroxy)-hexene-3 in respect of 100 wt. parts of said polymer, and an electric conductive substance.

If required, age resistors, processing aids and the like may be further added thereto according to the operation conditions.

As the result of researches by the inventors it has been confirmed that the amount of carbon black (25-70 wt. parts based on 100 wt. parts of the polymer), amine-, or phenol-based age resistors and zinc stearate and the like processing agents do not affect the ease of stripping off the semiconductive layer.

An example of the insulated cable having the external semiconductive layer of the invention is shown in FIG. 1, wherein, the cable consists of the conductor 1, internal semiconductive layer 2, insulating layer 3 and external semiconductive layer 4.

Examples of the invention, examples for reference and examples for comparison will be given hereinafter, in which different materials as mentioned hereinabove were used.

A stranded conductor having a sectional area of 100 mm<sup>2</sup> was covered with an ordinary extruded semiconductive layer, over which the insulating layer and semiconductive layer as shown in Table 1 were extruded in succession to cover the cable, and the product was completely crosslinked in a saturated water vapor under an atmospheric pressure of 15 atmospheres.

Incisions, 10 mm wide and running in the axial direction of the cable, were made in the external semiconductive layer covering the surface of the cable, and the cable was subjected to a peeling test by a tension tester, results of which are also shown in Table 1.

The semiconductive layers in the table respectively contained 50 wt. parts of acetylene carbon black, 1 wt. part of age resistor and 1 wt. part of zinc stearate, all based on 100 wt. parts of the base polymer, but the type and amount of the crosslinking agents and the thickness of the semiconductive layer were varied.

As is evident from the examples, only when an ethylene vinyl acetate copolymer containing 25-55 wt percent vinyl acetate and 2,5-dimethyl-2',5'-di(tertiary butyl peroxy)-hexene-3 are combined is the desired semiconductive layer of the present invention obtained, one which can be easily stripped off the base insulation of crosslinked polyethylene copolymer.

If the content of vinyl acetate is less than 25 wt. percent of the ethylene vinyl acetate copolymer, the layer will not be stripped off easily, and if it exceeds 55 wt. percent, its adhesion to the insulating layer will be impaired, making the cable unfit for use. When the content of vinyl acetate of the EVA copolymer is 25-55 wt. percent the layer can be stripped off with utmost ease. When the content of 2,5-dimethyl-2',5'-di(tertiary butyl peroxy)-hexene-3 is less than 0.2 wt. part based on 100 wt. parts of said copolymer, the peeling strength of the semiconductive layer is relatively low, and if it exceeds 6 wt. parts the adhesion of the semiconductive layer to the insulating material is impaired, also reducing the applicability of the cable. A range, in excess of 0.2 but less than 6 wt. parts, exhibits the best results.

As regards the thickness of the layer, if the thickness of the semiconductive layer extruded over the insulat-

TABLE I

| No.          | Insulating layer                                                             | Base polymer                                             | Semiconductive layer (over insulating layer) |                 | Peeling strength (kg./10 mm.)                  |
|--------------|------------------------------------------------------------------------------|----------------------------------------------------------|----------------------------------------------|-----------------|------------------------------------------------|
|              |                                                                              |                                                          | Crosslinking agent                           | Thickness (mm.) |                                                |
| Reference 1  | Polyethylene Sp. gr.=0.92 g./cc., *-3 MI=2, *-4 DCP=2.0%, age resistor=0.2%. | EVA*-1, VA=15%, MI=6                                     | X*-2, 1%...                                  | 0.5             | More than 5, and left on insulating layer.     |
| Example 1    | Same as Reference 1                                                          | EVA, VA=25%, MI=6                                        | X, 1%...                                     | 0.5             | 3.9.                                           |
| Example 2    | do                                                                           | EVA, VA=35%, MI=6                                        | X, 1%...                                     | 0.5             | 3.5.                                           |
| Example 3    | do                                                                           | EFA, VA=50%, MI=6                                        | X, 1%...                                     | 0.5             | 2.                                             |
| Reference 2  | do                                                                           | Same as Example 2                                        | Nil...                                       | 0.5             | Semiconductive layer torn so not stripped off. |
| Reference 3  | do                                                                           | do                                                       | X, 0.2%...                                   | 0.5             | Do.                                            |
| Example 4    | do                                                                           | do                                                       | X, 0.3%...                                   | 0.5             | 3.5.                                           |
| Example 5    | do                                                                           | do                                                       | X, 0.5%...                                   | 0.5             | 3.5.                                           |
| Example 6    | do                                                                           | do                                                       | X, 1.0%...                                   | 0.5             | 3.5.                                           |
| Example 7    | do                                                                           | do                                                       | X, 5.0%...                                   | 0.5             | 3.0.                                           |
| Reference 4  | do                                                                           | do                                                       | X, 6.0%...                                   | 0.5             | 0.3.                                           |
| Reference 6  | do                                                                           | do                                                       | X, 1.5%...                                   | 0.1             | Semiconductive layer torn so not stripped off. |
| Example 8    | do                                                                           | do                                                       | X, 1.5%...                                   | 0.2             | 3.3.                                           |
| Example 9    | do                                                                           | do                                                       | X, 1.5%...                                   | 0.5             | 3.4.                                           |
| Example 10   | do                                                                           | do                                                       | X, 1.5%...                                   | 1.0             | 3.3.                                           |
| Example 11   | Polyethylene Sp. gr.=0.92 g./cc., MI=4, DCP=2.0%, age resistor=0.2%.         | do                                                       | X, 2.0%...                                   | 0.7             | 3.5.                                           |
| Example 12   | Composition of Example 11: 100 wt. parts plus talc: 30 wt. parts.            | do                                                       | X, 2.0%...                                   | 0.7             | 3.0.                                           |
| Example 13   | Composition of Example 12: 100 wt. parts plus clay 30 wt. parts.             | do                                                       | X, 2.0%...                                   | 0.7             | 3.1.                                           |
| Example 14   | EVA, VA=16%, MI=3, DCP=2%, A.R.=0.2%.                                        | do                                                       | X, 1.5%...                                   | 1.0             | 4.3.                                           |
| Example 15   | Composition of Example 14: 100 wt. parts plus talc 30 wt. parts.             | do                                                       | X, 1.5%...                                   | 1.0             | 3.9.                                           |
| Comparison 1 | Same as Reference 1                                                          | do                                                       | DCP, 1.0%...                                 | 0.5             | More than 5, and left on insulating layer.     |
| Comparison 2 | do                                                                           | do                                                       | DCP, 5.0%...                                 | 0.5             | Do.                                            |
| Comparison 3 | do                                                                           | Same as Example 2 except EVA was replaced with DPD-6169. | X, 1.0%...                                   | 0.5             | Do.                                            |
| Example 16   | do                                                                           | EVA, VA=35%, MI=1                                        | X, 1%...                                     | 0.5             | 3.5.                                           |
| Example 17   | do                                                                           | EVA, VA=50%, MI=20                                       | X, 1%...                                     | 0.5             | 3.5.                                           |
| Example 18   | do                                                                           | EVA, VA=50%, MI=60                                       | X, 1%...                                     | 0.5             | 2.                                             |

\*-1 EVA=Ethylene vinyl acetate copolymer; VA=amount of vinyl acetate in copolymer.

\*-2 X=2,5-dimethyl-2',5'-di(tertiary butyl peroxy)-hexine-3.

\*-3 MI=Melt-flow index (g./10 min.) (ASTM-D-1238).

\*-4 DCP=Di- $\alpha$ -cumyl peroxide.

\*-5 DPD-6169=Ethylene ethylacrylate copolymer of UCC, USA.

ing layer is less than 0.1 mm, the layer, when stripped, will easily tear off, and it should be desirably more than 0.1 mm.

Thus, only when an ethylene vinylacetate copolymer containing 25-55 wt. percent vinyl acetate, and a range in excess of 0.2 but less than 6 wt. parts, of 2,5-dimethyl-2',5'-di(tertiary butyl peroxy)-hexine-3, based on 100 wt. parts of said copolymer, composes the semiconductive layer, will the semiconductive layer of the present invention, which can be stripped off completely with the utmost ease, be obtained. When crosslinking agents other than the aforementioned are used, such an excellent stripping effect as explained can not be obtained, as provided by the experiments of the inventors.

It was also confirmed when said crosslinking agent, 2,5-di-methyl-2',5'-di(tertiary butyl peroxy)-hexine-3 is added to a high molecular polymer other than ethylenevinylacetate copolymer, excellent effects can not be expected. Only by the use of the composition of the invention, can the semiconductive layer, which can be effectively stripped off, be obtained. The amount of carbon black is not particularly limited, but if it is less than 25 percent, the electric conductivity as required in the invention can not be obtained while an amount exceeding 70 percent will deteriorate the mechanical properties of the conductive layer, itself, impairing workability thereof, so that a range of 25-70 percent is desirable.

The present invention can be, of course, applied to electric cables having a insulating layer whose principal component is crosslinked polyethylene or crosslinked polyethylene copolymer, irrespective of the size and use of the cable.

#### What we claim is:

1. An insulated electric cable having an external semiconductive layer extruded over the insulating layer thereof comprising a cable insulated primarily with an insulation selected from the group consisting of cross-linked polyethylene and crosslinked polyethylene copolymer, and an external semiconductive layer consisting of an ethylene vinyl acetate copolymer containing 25-55 wt. percent vinyl acetate and 2,5-dimethyl-2',5'-di(tertiary-butyl/peroxy)-hexine-3 and an inclusion of an electric conductive substance.

2. An insulated cable as claimed in claim 1, wherein the insulating layer is made of crosslinked polyethylene.

3. An insulated cable as claimed in claim 1, wherein the insulating layer is made of a crosslinked polymer consisting of a copolymer of ethylene and vinyl acetate.

4. An insulated cable as claimed in claim 1, wherein inorganic filler is added to the insulating layer thereof.

5. An insulated cable as claimed in claim 1, wherein a range, in excess of 0.2 but less than 6 wt. parts, of 2,5-dimethyl-2',5'-di(tertiary butyl/peroxy)-hexine-3, based on 100 wt. parts of said ethylene vinyl acetate copolymer is contained in the semiconductive layer.

6. An insulated cable as claimed in claim 1, wherein the thickness of the external semiconductive layer is more than 0.1 mm.

7. An insulated cable as claimed in claim 1, wherein 25-70 wt. parts of carbon black based on 100 wt. parts of said copolymer is contained in the external semiconductive layer.

\* \* \* \* \*